

## UNITED STATES PATENT OFFICE

2,579,369

ADDITION ALLOY FOR TREATMENT  
OF STEEL

Charles N. Dawe, Detroit, Mich., assignor to Vanadium Corporation of America, New York, N. Y., a corporation of Delaware

No Drawing. Application September 13, 1948,  
Serial No. 49,119

9 Claims. (Cl. 75—138)

1

This invention pertains to a composition of matter used to improve the properties of ferrous metals and particularly of carbon and low alloy steels. It is especially effective in improving the balance of physical properties of steels ranging from .05% to 1.00% carbon, either with incidental alloying elements or with specified alloying elements up to 6% content by weight of the steel though its use is not limited thereto. This application is a continuation in-part of application Serial No. 623,169, filed October 18, 1945, now abandoned.

When a steel of proper composition is cooled rapidly from within its hardening temperature range, for example by quenching in oil, water, or some other medium, those portions which are most rapidly cooled harden while those portions which cool more slowly, for example the center of a bar, harden to a lesser extent. The depth of hardening depends upon the temperature from which the bar is cooled, the nature of the cooling medium, and the composition and other characteristics of the steel itself. The hardening capacity of a given steel is referred to as its hardenability, and this, as is well known, increases as the carbon content and the amount of certain other elements in the steel are increased and also as the grain size of the steel is increased (i. e., coarsened).

There are, however, certain advantages for which it is desirable to maintain fine grain in a steel even though increased hardenability is desired. The novel alloy which I have invented will serve this dual purpose, namely, to increase the hardenability of steel while at the same time producing fineness of grain so valuable in commercial utilization of the steel for numerous purposes.

In steel production, whether in the open-hearth furnace or electric furnace, it is customary to obtain fine grain size by the addition of about one pound or more of aluminum per ton of steel, depending on the composition and the steel-making process employed. The aluminum, having an affinity for oxygen greater than that of most other elements, must be added late in the melting operation and just before the steel is cast, so as to avoid possible loss of its grain refining properties. In open-hearth furnace manufacture it is customary to add the aluminum to the ladle while the heat is being tapped, but in the electric furnace the aluminum addition may be added either to the ladle or to the furnace just before tapping. As the amounts of aluminum are increased, within limits for a given

2

type of steel, the grain size becomes finer and to this extent the hardenability is diminished. Grain refinement is accompanied by greater uniformity of composition and by smaller variations in mechanical properties of castings or of bars, plates, and other shapes rolled or forged from the ingots.

Fineness of grain is often specified along with high hardenability in order to obtain the accompanying benefits of uniformity of composition and uniformity of properties. The combination of fine grain and high hardenability is generally obtained by the addition of aluminum, together with the addition of alloying elements (usually a combination of several) designed to increase the depth of hardness. Some of these elements are easily oxidized in the steel bath and at the same time are rather difficult to melt or cause to diffuse. This may be due to the fact that the required temperatures are too high or because such an amount of the elements must be added to bring about the desired effect upon hardenability that, unless they can be added in the liquid state, they cool the molten steel to such an extent that its manufacture will be impeded or its quality impaired. It is necessary, therefore, to engage the skill of the steelmaker in adding these elements a sufficiently short time before tapping to prevent effective oxidation, but a sufficiently long time before tap to permit complete absorption by the steel.

The situation becomes critical in the case of elements such as titanium, zirconium, and boron where the heats of combination with oxygen and nitrogen are exceedingly high; and critical also, insofar as the use of boron is concerned, due to the exceedingly small amount of addition required (from about 0.0002 to 0.003 per cent of the steel weight) and the consequent effects of very low recovery or of segregation.

I have discovered that when certain of the alloying elements used to increase the hardenability of steel are dissolved or intimately dispersed in aluminum through combination in the molten state, the resulting composition of matter when added to steel in the proper amount will increase the hardenability of the steel, while simultaneously insuring against very low recovery and segregation of the added elements and at the same time refine the grain size. The liquefying temperature of such a composition is above that of aluminum, yet far below that of the ferro-alloys in which form the hardening elements are usually added so that the alloys of my invention are more easily absorbed by the

melt. At the same time they are sufficiently diluted so as to insure uniformity of distribution and easy diffusion throughout the molten steel.

Among the alloying elements which increase the hardenability of steel are manganese, nickel, chromium, molybdenum, vanadium, titanium, boron, zirconium and silicon. My invention relates, however, to vanadium, titanium, boron, and zirconium alone or in combination, as hereinafter more specifically described, as dispersed in aluminum and, if desired, accompanied by incidental amounts of manganese and silicon alone or in association. Some iron may also be added as a carrier.

I have discovered that the desired effects of increased hardenability in the presence of fine grain size are especially pronounced in steels with 0.05 to 1.00% carbon (preferably 0.05 to 0.65%) containing additionally either incidental alloying elements or specified alloying elements up to 6% content by weight of the steel though the alloy is also useful in the treatment of other ferrous metals. By the addition to steels in this composition range, while the molten state, of alloys containing between 35% and 65% aluminum, along with suitable combinations of boron, titanium, zirconium and vanadium, I have been able to develop large increases in hardenability along with the desired fine grain size while avoiding the usual large losses incident to the addition of these powerful hardeners.

In addition to the aluminum content, the alloy of my invention contains boron in all cases, this element being the most powerful of the hardening agents per unit of weight and the most difficult to add to steels in such manner as to insure uniformity of distribution along with high recovery in effective form. The novel alloy preferably contains one or both of the elements titanium and zirconium, elements which are also very difficult to add to steels without large losses, in total amount varying from about 5% to about 35%, but preferably in the range of 10% to 25% total. The boron content is ordinarily from about .02% to about 5% in these alloys; preferably, however, in the range 1.5% to 1.5%. For the absolute maximum contribution to hardenability and grain size with minimum losses and also to prevent the formation of reaction products which may be detrimental to steel quality, some vanadium is added to the alloy, the amount usually being in the range of 2% to 35%, preferably between 5% and 20%. The total of titanium, zirconium, boron, and vanadium does not ordinarily exceed 40% and is generally between 10 and 30%.

Usually as a result of the method of manufacture, though they may be purposely included, there is present in the alloy as a remainder of relatively minor significance one or more of the elements, manganese and silicon in an amount not to exceed about 30% of the total and preferably not over 20% of the total. It will be realized that both manganese and silicon may contribute to the hardenability of the finished steel, but with the amounts that can possibly be added when considering the fact that the gross weight of this alloy addition is usually about 1/2 to 2% of the steel weight this contribution to hardenability is relatively minor and insignificant.

The balance of the alloy is preferably iron which serves as a carrier for the other elements, and, of course, has the desirable property of a melting point no higher than that of the ferrous metal to which the alloy is added. Ordinarily the iron will be present in amount of from about 15% to 40%, though it will be understood that the precise

amount within or without this range is dependent upon the desired quantities of the other elements.

The alloy of my invention may be produced by any convenient method, either by direct aluminothermic reduction of oxides or other suitable compounds with an excess of aluminum present, or added after the reaction is complete; or it may be produced by silico-thermic reduction or by reduction with an electric arc using aluminum or silicon as reducing agents and operating on a bath of aluminum or aluminum-silicon alloy, or excess aluminum may be combined with the alloy after electric reduction. These are just examples of methods that may be employed and this description should not be interpreted as placing any limitation upon the mode of manufacture, which method is not considered to be part of this invention.

Alloys of the following percentage compositions are typical of my invention:

| Alloy | Al    | B    | Ti    | Zr    | V     | Si    | Mn    | Fe    |
|-------|-------|------|-------|-------|-------|-------|-------|-------|
| I     | 50.80 | 0.20 | 10.00 | ----- | 16.00 | ----- | ----- | 23.00 |
| II    | 41.00 | 0.20 | 13.20 | ----- | 8.60  | ----- | ----- | 37.00 |
| III   | 41.00 | 0.50 | 13.30 | 2.70  | ----- | 3.30  | 5.30  | 33.90 |
| IV    | 37.30 | 0.50 | 6.60  | 4.00  | 6.60  | 20.00 | ----- | 25.00 |

The weight of alloy per ton of steel varies ordinarily from about 2 to about 20 pounds but may in special cases reach more than twice the latter figure. The amount employed in any instance is dependent upon the composition of the steel, the steel making method, and the detailed results that it is desired to obtain, and, as those in the art will understand, it is adjusted in accordance with preliminary experience in each instance.

What is claimed is:

1. A grain refining and hardenability imparting agent for addition to molten steel consisting essentially of about 35-65% aluminum, about .02-5% boron, and about 5-35% of at least one of the elements selected from the group consisting of titanium and zirconium, the balance substantially all iron, said iron being not less than 15%.
2. A grain refining and hardenability imparting agent for addition to molten steel consisting essentially of about 35-65% aluminum, about .02-5% boron, and about 2-35% vanadium, the balance substantially all iron, said iron being not less than 15%.
3. A grain refining and hardenability imparting agent for addition to molten steel consisting essentially of about 35-65% aluminum, about .02-5% boron, about 5-35% of at least one of the elements selected from the group consisting of titanium and zirconium, about 2-35% vanadium, the balance substantially all iron, said iron being not less than 15%.
4. A grain refining and hardenability imparting agent for addition to molten steel consisting essentially of about 35-65% aluminum, about .02-5% boron, up to 30% of at least one of the elements selected from the group consisting of manganese and silicon, the balance substantially all iron.
5. A grain refining and hardenability imparting agent for addition to molten steel, consisting essentially of about 35-65% aluminum, about .02-5% boron, and the balance substantially all iron.
6. An agent for addition to molten steel consisting essentially of about 35 to 65% aluminum, about 0.02 to 5% boron, about 5 to 35% of one

or more elements selected from the group titanium and zirconium, and up to 30% of one or more elements selected from the group consisting of silicon and manganese, the balance substantially iron, said iron being not less than 15%.

7. An agent for addition to molten steel consisting essentially of about 35 to 65% aluminum, about 0.02 to 5% boron, about 2 to 35% vanadium and up to 30% of at least one of the elements selected from the group consisting of silicon and manganese, the balance substantially iron.

8. An alloy for addition to molten steel and effective in increasing the hardenability and refining the grain size of the steel composed of about 35 to 65% aluminum, about 0.02 to 5% boron, about 5 to 35% of at least one of the elements selected from the group consisting of titanium and zirconium, about 2 to 35% vanadium, and up to about 30% of an element selected from the group consisting of silicon and manganese, the remainder being iron and incidental impurities, said iron being at least 15%.

9. An alloy for addition to molten steel and effective in increasing the hardenability and re-

fining the grain size of the steel consisting essentially of about 35 to 65% aluminum, about 0.02 to 5% boron, about 5 to 35% of at least one of the elements selected from the group consisting of titanium and zirconium, about 2 to 35% vanadium, the total of said boron, titanium, zirconium, and vanadium being less than 40%, up to about 30% of an element selected from the group consisting of silicon and manganese, and about 15 to 40% iron.

CHARLES N. DAWE.

#### REFERENCES CITED

The following references are of record in the file of this patent:

#### UNITED STATES PATENTS

| Number    | Name     | Date           |
|-----------|----------|----------------|
| 2,291,842 | Strauss  | Aug. 4, 1942   |
| 2,295,706 | Comstock | Sept. 15, 1942 |

#### FOREIGN PATENTS

| Number  | Country | Date         |
|---------|---------|--------------|
| 478,462 | Germany | July 2, 1929 |